

3,838,022  
**CHELATING/COMPLEXING DIP IN BRIGHT  
PLATING OF BRASS**

Michael G. Bartolini, Southbury, and Edmund E. Horner,  
Watertown, Conn., assignors to MacDermid Incorporated,  
Waterbury, Conn.  
No Drawing. Filed Nov. 9, 1972, Ser. No. 305,005  
Int. Cl. C23b 5/62

U.S. Cl. 204—32 R

8 Claims

## ABSTRACT OF THE DISCLOSURE

Process of nickel plating brass-type copper alloys. The conventional plating cycle steps of (1) soak clean, (2) electroclean (as a single or two separate step operation), (3) acid dip and (4) then electroplate, are modified by incorporating an additional step consisting in immersing the copper alloy substrate in an aqueous chelating/complexing solution after the soak clean but before the acid dip steps. The purpose is to eliminate visible irregularities in the nickel deposit, as well as to improve adhesion of the plate to the substrate. The preferred chelating/complexing materials in aqueous solution include the alkali metal salts of polycarboxylic acids, such as gluconic, tartaric, heptonic, oxalic and citric; the alkali metal salts of polyphosphoric acids; the alkali metal salts of lower alkyl-substituted amino acetic acids and hydroxy amino acids; and compatible combinations of such agents.

## SUMMARY OF THE INVENTION

### Field of Invention

The invention is directed to improving the surface uniformity and specular appearance as well as the adhesion of nickel electroplates, more particularly bright nickel electroplates, on brass-type copper alloy substrates.

### PRIOR ART

Brass and related copper-tin-zinc-lead alloys are by far the most difficult metal substrates to electroplate properly in order to produce a finish which is free of visual or optical irregularities such as clouding, haze or striation, as well as being free of mechanical irregularities such as poor adhesion and blistering. Nickel electroplate and especially decorative bright nickel deposits are most troublesome in respect to clouding, etc. and poor adhesion. It is well known that copper alloys containing zinc, lead and tin are substantially more troublesome in this respect than is copper itself when used as a base or substrate metal; yet for better physical properties, such as castability or free machining, the alloying components are a practical necessity in the substrate.

Various attempts have been made heretofore to overcome clouding, haze, striation, as well as poor adhesion, in nickel plated brass substrates. The problem of objectionable patterns in the finished surface is often emphasized or exaggerated by final chromium plating of nickel plated buffed brass parts, and frequently these do not appear until the last stage of manufacture has been completed. Such defects in surface characteristics naturally cause the parts to lose esthetic appeal and require their rejection even if mechanically the finish is satisfactory.

Attempts to improve the results have been directed toward varying concentrations, temperatures, current densities, immersion times, as well as compositions, in the various treatment solutions generally employed in the normal pretreatment and electroplating operations. Since the number of operations involved in the normal cycle is substantial, the permutations and combinations possible in the way of changes that can be made become quite complex, and their coordination is largely a matter of em-

pirical determination. This will be more evident from the following outline of steps usually involved in the typical preparation and plating cycle for a brass or similar brass-type copper alloy substrate:

5 Conventional preparation and plating cycle steps

(a) Soak clean, 1 to 5 minutes at 160°–200° F. in a proprietary alkaline cleaner, such as a moderately alkaline solution of borax, pyrophosphate, soap, ethoxylated non-ionic surfactant, a small amount of organic chelating agent, dispersing agent and suitable water soluble solvent, such as ethylene glycol monobutyl ether. Such a cleaner is conventionally used at a concentration, for example, of about 8 ozs./gal.

(b) Following a thorough water rinse, electroclean the substrate in any suitable proprietary composition, such as a solution of soda ash, sodium metasilicate glassy phosphate, sodium hydroxide and a minor amount of anionic surfactant at a concentration of about 8 ozs./gal. for 10 to 30 seconds at 140°–160° F. wherein the part is made anodic or cathodic or a combination of cathodic and anodic, using potentials to give a current density of 25 ASF.

(c) Again following a thorough water rinse, the electroclean step is repeated, generally in a second and completely separate tank, but under the same operating conditions as used in the first such treatment.

(d) After another water rinse, the part is given an acid clean treatment in a proprietary acid salt solution, such as a mixture of sodium bisulfite and ammonium persulfate, or regular mineral acid solution, typically for 1 to 5 minutes at 200° F., at an acid salt or equivalent mineral acid concentration of from 1 to 8 ozs./gal.

(e) Finally, after still another thorough water rinse, the substrate is made the cathode in a plating tank containing a proprietary nickel electrolyte and plated with a bright nickel deposit. Conventionally, too, a further protective thin chromium plate is deposited in a subsequent plating step.

40 Thus there are many possibilities for change which can and do affect the end result, some of which have been investigated and their results are generally predictable, but many of which cannot be anticipated or rationalized.

The present invention rests on a discovery involving modification of the conventional cycle of operations above outlined to incorporate a step of immersing the substrate metal part in an aqueous solution of a water-soluble organic chelating/complexing agent, or combination of such agents. It is an important aspect of the present discovery that such chelating/complexing solution treatment follow the soak cleaner step and precede the electroclean step (or the first of such steps if two are employed); or alternatively that the chelating/complexing treatment step follow the electrocleaner (or replace the second electroclean operation if two are employed) and precede the acid clean treatment.

When this modification is employed, as more fully described below, the degree of improvement is so remarkable with respect to depth, clarity and uniformity of final electroplate as to lead those skilled in the art to conclude that the bright nickel plating operation has been extensively modified, whereas this is not so.

The reason for the improvement afforded by the invention is not fully understood. Therefore, without intending the following explanation to be binding, it is postulated that much of the difficulty encountered in the normal processing cycle of steps described above is due to reactions between some of the alloying metals of the copper substrate and buffing or polishing compounds used in mechanically preparing the substrate surface. Such reactions are capable of producing trace amounts of metal

soaps and/or other insoluble metal compounds on the surface of the substrate. These trace amounts of insoluble compounds probably become trapped and are not readily removed by the sequence of treatments heretofore normally employed. However, with the incorporation of the chelating/complexing treatment step taught by this disclosure, the modified process is quite effective in solubilizing and removing the postulated insoluble surface film to a greater degree than has usually been accomplished heretofore.

As mentioned above, there is some criticality to the order of treatment steps to attain the best results; for example, merely adding an otherwise satisfactory chelating/complexing agent to the soak cleaner or to the electro-cleaner treatment tank, as might appear reasonable, does not produce the same order of improvement as where a separate chelating/complexing treatment step is utilized. Presumably some competing reaction occurs if such a combined soak cleaner/chelator or electroclean/chelator combination is attempted, with resulting loss of effectiveness of the chelating agent.

Specific chelating or complexing agents found to be useful in the practice of the invention include the following:

- (a) Tetrasodium (and potassium and ammonium) pyrophosphate.
- (b) Sodium (and potassium) tripoly phosphate.
- (c) Various alkaline salts of nitrilotriacetic acid (NTA), including the sodium, potassium, lithium and ammonium salts.
- (d) Similar alkaline salts of hydroxyethyl ethylenediamine triacetic acid (HEDTA).
- (e) Similar alkaline salts of diethylenetriamine pentaacetic acid (DTPA).
- (f) Similar alkaline salts of ethylenediamine tetraacetic acid (EDTA).
- (g) Similar alkaline salts of N,N-dihydroxyethyl aminoacetic acid.
- (h) Similar alkali metal salts of gluconic, tartaric, heptonic, oxalic and citric acids.
- (i) Amines such as ethylenediamine, triethanolamine, and diethylene triamine.
- (j) Trisodium salt of aminotrimethyl phosphoric acid.

Certain combinations of the foregoing agents, which are not incompatible in respect to the substituent groupings, are quite effective and sometimes preferred. Thus a combination of sodium gluconate and the tetra sodium salt of ethylenediamine tetraacetic acid is especially satisfactory.

With regard to operative conditions of use of the chelating/complexing solution, it has been found that very dilute concentrations of the agents in aqueous solution produce substantial improvement. While minimum effective concentration will of course depend on the particular agent or combination of agents employed, as well as the factors of time of immersion and temperature of the solution, in general at least about 0.002 molar concentration is required. It is preferred, however, for practical operations to employ a higher concentration, usually in the range of about 0.01 molar to 0.02 molar. Some better understanding of the concentration factor can be obtained from the specific examples given below for illustration purposes. There is apparently no criticality as to maximum concentration of the chelating/complexing agents in solution so far as operability is concerned. Rather, the upper concentration limit is determined by solubility and economic factors.

The temperature of the chelating/complexing solution, and the time of immersion, are naturally interrelated in a generally inverse order. For industrially useful operations, a minimum temperature of at least 45° F. is required, while the maximum is just below boiling. The preferred condition is within the range of 125° F. to 155° F. This corresponds with an immersion time of about 30 seconds to one minute, which again is determined by practical conditions. Immersion times may however be

varied from as little as 5 seconds up to at least 10 minutes, with appropriate adjustment in solution temperature and concentration.

The parameters within which successful practice of the invention is possible are illustrated by the following examples of some specific preplating preparation and plating cycles.

#### Example 1

The conventional preparation and plating cycle of steps 10 above described is followed, with the exception that the second electrocleaning operation, step (c), is replaced by treatment of the metal part in an aqueous solution of sodium gluconate and the tetra-sodium salt of ethylenediamine tetraacetic acid. An approximate weight ratio of 15 2 parts gluconate salt to 1 part EDTA salt (tetrasodium) is employed, with a total concentration of the two of about 2 ounces per gallon of solution. The foregoing solution represents the optimum concentration condition and some variation is possible. In general, the preferred range of 20 complexer bath composition consists of about 1% to 10% by volume of a concentrate comprising 60% by weight of water, 30% by weight of sodium gluconate and 10% by weight of the tetrasodium salt of EDTA.

The temperature of the solution is maintained at 120°- 25 130° F. and the brass parts to be plated are immersed in this for about 30 seconds. After this chelator/complexer step, the parts are given the standard acid clean, as specified in the conventional process, followed by nickel plating and the deposition of a thin protective chromium plate.

The resulting parts exhibit a specular surface free of haze, clouds and striations, and the electrodeposited metal has excellent adherence to the brass without any evidence of blisters.

35 As a variation of this procedure, the chelator/complexer solution may be maintained at room (75° F.) temperature, in which case the parts are immersed in it for about 1 minute. At still lower temperature (45° F.) of the chelator/complexer, it is still effective but the time of immersion must be increased substantially, generally to around 10 minutes.

#### Example 2

The procedure of Example 1 is duplicated with the exception that the chelator/complexer solution contains only sodium gluconate, at a concentration of 4 ounces per gallon. At a solution temperature of 120° F., good clear nickel plated deposits are obtained using a 30 second dip in the chelator/activator solution, and still better results are obtained if the immersion time is increased to 1 minute.

#### Example 3

The same procedure was followed as in Example 1, except that the chelator/complexer solution consisted of a 5% (volume) aqueous solution of "Dequest 2006." This is a chelating agent consisting of amino methyl sodium salt of phosphoric acid, produced by Monsanto Co. At a solution temperature of 120° F. and an immersion time of 30 seconds, haze-free, adherent nickel plated deposits are uniformly obtained on the brass substrates.

Substituting "Dequest 2001" for the material above does not give wholly satisfactory results because of attack of the brass. This material is an acid form of "Dequest 2006."

#### Example 4

The procedure of the foregoing example is repeated using an aqueous solution of the tri-sodium salt of nitrilotriacetic acid. At a concentration of 4 oz./gal. and a solution temperature of about 120° F., excellent plate deposits are obtained with an immersion time of 30 seconds in the chelator/complexer bath.

At a solution temperature of 160° F., 30 second immersion, the resulting plated deposit is clear and bright, even though some tarnishing of the brass substrate ap-

pears. Decreasing the solution temperature to 75° F., still retaining a 30-second immersion time also gives excellent results in respect to plated deposit clarity, brilliance and adhesion. No tarnishing of the brass is apparent in this case.

Modification of the concentration of the chelator concentration, as by reducing it in half, does not noticeably affect the finish where the solution is maintained at 120° F. At lower temperatures, some increase in immersion time appears beneficial. Somewhat less tendency for tarnishing of the substrate brass surface is noted at the lower pH condition resulting from decrease in the concentration of the agent.

#### Example 5

The procedure is repeating using "Hampshire DEG" as the chelator/complexer agent. This is an anionic liquid sequestrant sold by Hampshire Chemical, Div. of W. R. Grace & Co., Nashua, N.H., and consists essentially of sodium dihydroxyethyl glycine. A 5% (vol.) solution of this agent in water, at a temperature of 120° F., gives excellent results on 30 second immersion cycle. Reducing the concentration to around 2% (vol.) at the same temperature still provides entirely satisfactory finish in the nickel plate. At the lower concentration but raising the bath temperature to 160° F., some tarnishing of the brass substrate appears, however the final nickel plate finish is still excellent.

#### Example 6

The procedure is repeated using diethylenetriamine at a concentration of 2% (vol.) in aqueous solution at 120° F. for 30 seconds. A satisfactory final nickel finish is obtained which, however, does not appear quite as bright and clear as in some of the preceding examples. Operation of this solution at higher temperature, e.g. 160° F., shows some increase in tarnish in the brass substrate prior to plating but does not appear substantially to affect the final nickel finish.

#### Example 7

The several alkali metal salts of ethylenediamine tetra-acetic acid also produce satisfactory results when used as chelator/complexer agents in the novel process. "Hampene-Na<sub>4</sub>," "Hampene-Na<sub>3</sub>," and "Hampene-Na<sub>2</sub>" (all Hampshire Chemical, Div. W. R. Grace & Co.), the various hydrated sodium salts of EDTA, as well as "Hampene-215" the technical tetrasodium salt, all produce a bright clear finish when used in concentrations of from 2 to 5 ounces/gal. at 120°-130° F.

#### Example 8

Diethylene triamine penta acetic acid pentasodium salt, available commercially as "Hamp-Ex80," is also suitable for use as a chelator/complexer agent in the process of the invention. The same concentration range (approximately 2 to 5 oz./gal.), at the same temperature conditions (120°-130° F. preferred, but operative up to at least 160° F.) for similar immersion times give clear, bright final nickel plated finishes.

#### Example 9

Another suitable agent is the trisodium salt of N-hydroxyethyl ethylenediamine triacetic acid. This is available commercially as "Hamp-OL Crystals" and the "Hamp-OL 120," a liquid. Use of these in amounts of 2 to 5 oz./gal. of the crystalline material, or 5% (vol.) of the liquid, produce a bright, specular finish in the final nickel plated brass substrate.

#### Example 10

Sodium tripolyphosphate, tetrasodium pyrophosphate, 70 sodium hexametaphosphate, and to somewhat lesser extent, trisodium orthophosphate, can be used alone as the chelator/complexer in the practice of the invention. Satisfactory results are obtained at concentrations of 2 to 5 oz./gal. It is usually necessary with these to operate at 75

higher temperatures, generally at least 160° F. to get comparably good results.

#### Example 11

5 The alkaline salts of carboxylic acids in addition to gluconic are also operative. Sodium tartrate, sodium heptonate, sodium oxalate and sodium citrate each performs similarly to the gluconate. These may be used in combinations with each other or with other complexing agents mentioned above. The concentrations and other conditions of operation are generally the same as above described.

10 In all cases a more uniform result is obtained over a longer period of use of the chelator/complexer bath where a thorough water rinse of the brass parts is provided ahead of the complexing agent. It is also preferable to have a water rinse immediately following the complexing agent treatment.

15 In each of the examples above, the chelator/complexer was used after an electroclean treatment. The procedure will also work where the chelator/complexer step immediately follows the soak clean (and a water rinse) and precedes the electroclean step. The conditions as to concentration, temperature and time remain as before.

20 What is claimed is:

25 1. In the method of nickel plating a substrate surface composed of a copper alloy containing zinc, tin, lead or combinations thereof, wherein the plating cycle includes immersing the substrate successively in conventional soak cleaner, electrocleaner and acid clean solutions, followed by electrodeposition of the nickel, the improvement which comprises: immersing the substrate in an aqueous solution of a chelating/complexing agent after the soak cleaner but before the acid cleaner steps in said cycle.

30 2. The method of claim 1, wherein the chelator/complexer immersion step follows the soak clean but precedes the electroclean step.

35 3. The method as defined in claim 1, wherein the complexer immersion step follows the electroclean but precedes the acid clean step.

40 4. The method of claim 1, wherein the substrate is immersed in the chelator/complexer solution for a period of 5 seconds to 10 minutes at a solution temperature of from 45° F. to just below boiling, said complexer solution being from at least about 0.002 molar up to the limit of saturation in respect to said chelator/complexer agent.

45 5. The method of claim 4, wherein the period of immersion in said complexer solution is about 30 seconds to 1 minute at a solution temperature of about 125° to 155° F. and the concentration of complexing agent is about 0.010 molar to 0.020 molar in said chelator/complexer agent.

50 6. The method of claim 4, wherein said aqueous concentrate of said complexer consists of about 1% to 10% by volume of a concentrate comprising 60% by weight of water, 30% by weight of sodium gluconate and 10% by weight of the tetrasodium salt of EDTA.

55 7. The method as defined in claim 1, wherein said complexing agent is a member selected from the group consisting of

A. sodium, potassium and ammonium salts of pyrophosphates and sodium and potassium salts of polyphosphates

B. sodium, potassium and ammonium salts of lower alkyl carboxylic acids

C. sodium, potassium and ammonium salts of amino and hydroxy-amino substituted lower alkyl carboxylic acids, and

D. lower alkyl substituted amines.

60 8. The method as defined in claim 1, wherein said complexing agent is a member selected from the group consisting of

A. sodium, potassium and ammonium pyrophosphates and sodium and potassium tripolyphosphates;

- B. sodium, potassium and ammonium salts of gluconic, tartaric, heptonic, citric and oxalic acids;
- C. sodium, potassium and ammonium salts of nitrilo-triacetic, hydroxyethyl ethylenediamine triacetic, di-ethylene triamine pentaacetic, ethylenediamine tetra-acetic and dihydroxyethyl aminoacetic acids;
- D. ethylenediamine, triethanol amine and diethylene triamine;  
and mixtures thereof.

**References Cited****FOREIGN PATENTS**

1,421,965 11/1968 Germany 204—29

5 JOHN H. MACK, Primary Examiner  
W. I. SOLOMON, Assistant Examiner**U.S. CL. X.R.**

10 204—29, 49